



US008342213B2

(12) **United States Patent**  
**Sutton et al.**

(10) **Patent No.:** **US 8,342,213 B2**  
(45) **Date of Patent:** **Jan. 1, 2013**

(54) **METHOD FOR MANUFACTURING A TURF REINFORCEMENT MAT**

(75) Inventors: **Alan Sutton**, Gainesville, GA (US); **Rebecca Page**, Flowery Branch, GA (US); **George Miles Gibby**, Cornelia, GA (US)

(73) Assignee: **Lumite, Inc.**, Alto, GA (US)

(\*) Notice: Subject to any disclaimer, the term of this patent is extended or adjusted under 35 U.S.C. 154(b) by 189 days.

(21) Appl. No.: **12/845,234**

(22) Filed: **Jul. 28, 2010**

(65) **Prior Publication Data**

US 2011/0027540 A1 Feb. 3, 2011

**Related U.S. Application Data**

(60) Provisional application No. 61/229,962, filed on Jul. 30, 2009.

(51) **Int. Cl.**

**D03D 3/08** (2006.01)  
**D03D 11/02** (2006.01)  
**D03D 41/00** (2006.01)  
**D03D 25/00** (2006.01)

(52) **U.S. Cl.** ..... **139/384 R**; 139/304; 139/309; 139/11

(58) **Field of Classification Search** ..... 139/11, 139/304-316, 383 R, 384 R, 387 R, DIG. 1  
See application file for complete search history.

(56) **References Cited**

**U.S. PATENT DOCUMENTS**

2,757,434 A \* 8/1956 McCord et al. ..... 28/156  
3,047,444 A \* 7/1962 Harwood ..... 428/153

3,279,221 A \* 10/1966 Gliksmann ..... 66/192  
3,696,623 A \* 10/1972 Heine et al. ..... 405/19  
4,002,034 A \* 1/1977 Muhring et al. ..... 405/19  
4,183,993 A \* 1/1980 Benstead et al. ..... 442/314  
4,421,439 A \* 12/1983 ter Burg et al. ..... 405/302.7  
4,472,086 A \* 9/1984 Leach ..... 405/302.7  
4,619,120 A \* 10/1986 Markowitz ..... 66/192  
4,790,691 A \* 12/1988 Freed ..... 405/263  
4,837,387 A \* 6/1989 van de Pol ..... 442/185  
4,957,390 A \* 9/1990 Shoesmith ..... 404/70  
4,992,003 A \* 2/1991 Perach ..... 405/302.7  
5,326,192 A \* 7/1994 Freed ..... 47/9  
5,567,087 A \* 10/1996 Theisen ..... 405/302.7  
5,612,114 A \* 3/1997 Zalewski et al. ..... 428/102  
5,616,399 A \* 4/1997 Theisen ..... 428/175  
5,795,835 A \* 8/1998 Bruner et al. ..... 442/310  
5,856,243 A \* 1/1999 Geirhos et al. ..... 442/57  
6,171,022 B1 \* 1/2001 Decker ..... 405/16  
6,305,875 B1 \* 10/2001 Matsumoto ..... 405/16  
6,368,024 B2 \* 4/2002 Kittson ..... 405/302.7  
6,429,153 B1 \* 8/2002 Welkers et al. ..... 442/35  
6,481,934 B1 \* 11/2002 Alexiew ..... 405/302.7  
6,503,853 B1 \* 1/2003 Kassner et al. ..... 442/57  
6,706,376 B1 \* 3/2004 Von Fransecky ..... 428/212

(Continued)

**FOREIGN PATENT DOCUMENTS**

WO 2007067833 A2 6/2007

*Primary Examiner* — Bobby Muromoto, Jr.

(74) *Attorney, Agent, or Firm* — Gardner Groff Greenwald & Villanueva, PC

(57) **ABSTRACT**

A turf reinforcement fabric and a method for producing such a fabric by weaving a plurality of filaments in a predetermined pattern to form a three-dimensional structure formed to have a loft thickness without the application of heat to heat shrink the fibers.

**19 Claims, 6 Drawing Sheets**



U.S. PATENT DOCUMENTS

|           |      |         |                  |           |              |      |         |               |        |
|-----------|------|---------|------------------|-----------|--------------|------|---------|---------------|--------|
| 6,877,932 | B2 * | 4/2005  | Prevost          | 405/38    | 7,820,560    | B2 * | 10/2010 | Weiser et al. | 442/32 |
| 7,279,436 | B2 * | 10/2007 | Pintz            | 442/43    | 2002/0157429 | A1 * | 10/2002 | Matsumoto     | 66/195 |
| 7,470,094 | B2 * | 12/2008 | Heathcott et al. | 405/302.7 | 2005/0287343 | A1   | 12/2005 | Weiser        |        |
| 7,699,949 | B2 * | 4/2010  | Newton et al.    | 156/60    | 2006/0134389 | A1   | 6/2006  | Weiser        |        |
| 7,786,026 | B2 * | 8/2010  | Newton et al.    | 442/2     | 2008/0220185 | A1 * | 9/2008  | Fan et al.    | 428/17 |

\* cited by examiner



FIG. 1



FIG. 2



FIG. 3



FIG. 4



This section repeats itself 98 times between selvages.

**FIG. 5**

**Harness Weave Pattern**

1. 9, 13 up
2. 10, 14 up
3. 9,11,13,14 up
4. 9,10, 12-14 up
5. 7, 9, 10, 11, 13, 14 up
6. 6, 8-14 up
7. 3, 5 ,7,9-14 up
8. 4,6-14 up
9. 3,5,7-14 up
10. 3,4,6-14 up
11. 3,4,6-14 up
12. 3,4,6-14 up
13. 3,4,5,7-14 up
14. 3,4,6-14 up
15. 3,5,7-14 up
16. 4,7-14 up
17. 3,5,7,9-14 up
18. 8-14 up
19. 7,9-11,13,14 up
20. 9,10,12,13,14 up
21. 9,11,13,14 up
22. 10,13,14 up
23. 9,13 up
24. 14 up
25. 13 up
26. 14 up
27. 14 up
28. 14 up

**FIG. 6**



FIG. 7

## METHOD FOR MANUFACTURING A TURF REINFORCEMENT MAT

### CROSS-REFERENCE TO RELATED APPLICATION

This application claims priority benefit to U.S. Provisional Patent Application Ser. No. 61/229,962, filed Jul. 30, 2009, which is hereby incorporated herein by reference in its entirety.

### TECHNICAL FIELD

The present invention relates generally to the fields of woven materials and turf management, and more particularly to a method of manufacturing fabrics for the reinforcement of natural turf.

### BACKGROUND OF THE INVENTION

According to the U.S. Environmental Protection Agency (EPA), high volume and high velocity storm water runoff can erode soil within the open channels, drainage ditches, and swales, and on steep exposed slopes, increasing the transport of sediments into receiving orders. Water quality impacts of increased sediment load include the conveyance of nutrient and pesticide pollutants, disruption of fish spawning, and impairment of aquatic habitat.

Traditionally, hard armor erosion control techniques such as concrete blocks, rock rip rap, and reinforced paving systems have been employed to prevent soil erosion in these highly erosive areas. Although these measures can withstand great hydraulic forces, they are costly, and they do not provide the pollutant removal capabilities of vegetative systems.

Turf reinforcement mats (TRMs) enhance the natural ability of vegetation to permanently protect soil from erosion. TRMs are composed of interwoven layers of non-degradable geo-synthetic materials such as polypropylene, nylon and polyvinyl chloride netting, stitched together to form a three-dimensional matrix. They are thick and porous enough to allow for soil filling and retention. In addition to providing its scour protection, the mesh netting of TRMs is designed to enhance vegetative root and stem development. By protecting the soil from scouring forces and enhancing vegetative growth, TRMs raise the threshold of natural vegetation to withstand higher hydraulic forces on stabilization slopes, stream banks, and channels. In addition to reducing flow velocities, the use of natural vegetation provides particulate contaminant removal through sedimentation and soil infiltration, and improves the aesthetics of the site.

TRMs offer high shear strength, resistance to ultraviolet degradation, and resistance to chemicals found in soils. TRMs, unlike temporary erosion control products, are designed to stay in place permanently to protect seeds in soils and to improve germination. TRMs can incorporate natural fiber materials to assist in establishing vegetation. However, the permanent reinforcement structure of TRMs is composed of entirely non-degradable synthetic materials. A variety of ground anchoring devices can be used to secure TRMs, including: U-shaped wire staples, metal pins, and wood or plastic stakes. Appropriate ground anchoring devices are chosen based on site-specific soil and slope conditions.

The use of TRMs allows vegetative cover to be extended to areas where site conditions would otherwise limit it. This helps to establish and maintain a continuous vegetative cover throughout the applied area. TRMs can be applied to most sites or structures where permanent erosion control is

required. This technology has been effectively used in both urban and rural areas and in a variety of climactic conditions. Although most effective when used in fully vegetative areas, TRMs have been used to prevent erosion even in arid, semi-arid, and high altitude regions with limited vegetative growth. In these areas, vegetation establishment is slow or difficult, and the TRM matrix is typically filled with native soils for protection.

TRMs are being used to control erosion and stabilize soil to 10 control runoff from land disturbing activities with steep slopes, and to prevent scouring in storm water detention ponds, water storage ponds, small open channels, drainage ditches, and runoff conveyance systems within the parking lot medians, and along stream banks and shorelines.

15 In addition to their use for new construction projects, TRMs have been used to retrofit existing hard armor systems. In addition to improving water quality, TRMs can provide aesthetic enhancement, especially in areas lacking vegetative growth.

20 TRMs provide water quality benefits by allowing the growth of vegetation in areas where impervious conveyance systems would otherwise be used. In general, the performance of TRMs is closely tied to the vegetative establishment and growth. The performance of the TRM-lined conveyance system depends on the duration of the runoff event to which it is subjected.

Known TRM materials are woven in a pattern that when 25 exposed to heat, creates a loft or three-dimensional structure. In some instances, the loft must meet a minimum thickness specification (for example, 0.25 inch) in order to be considered a TRM. The energy required for heating the material, as well as the additional equipment required for carrying out the heating process, add considerably to the expense of the product. Also, the material typically shrinks in the lengthwise and 30 widthwise dimensions as the fibers contract during heat-treatment process to create the loft. Thus, a loom width wider than the desired final product width is typically required.

Known TRM materials also typically include a single fiber 35 or end at the peak and valley points of the weave pattern, and 40 provide inadequate compression resistance for some applications.

It is to the provision of an improved TRM product and manufacturing process that the present invention is primarily directed.

### SUMMARY OF THE INVENTION

In example embodiments, the present invention provides a 45 turf reinforcement mat and a method of manufacturing a turf reinforcement mat without the need for the application of heat. The particular weave pattern, tension and materials used in fabricating the material create a three-dimensional product. In example embodiments, the turf reinforcement mat has, for example, a 0.25 inch or greater loft/thickness.

50 In one aspect, the present invention relates to a three-dimensional turf-reinforcement fabric. The three-dimensional turf-reinforcement fabric includes a woven array of fibers comprising a first plurality of fibers arranged in a first direction and a second plurality of fibers arranged in a second direction generally perpendicular to the first direction. The woven array of fibers defines rows and columns of cells, wherein each cell comprises fiber segments of the first plurality of fibers and the second plurality of fibers being spaced at differing heights in a third direction perpendicular to the first and second directions. The three-dimensional turf-reinforcement fabric is formed without the application of heat to shrink the fibers and produce a loft.

In another aspect, the invention relates to a method of forming a three-dimensional turf-reinforcement fabric. The method includes weaving a first plurality of fibers arranged in a first direction and a second plurality of fibers arranged in a second direction generally perpendicular to the first direction into a woven array having fiber segments being spaced at differing heights in a third direction perpendicular to the first and second directions, without the application of heat to produce a loft.

In another aspect, the invention relates to a turf reinforcement mat including a weave formed of a plurality of warp fibers, a plurality of weft fibers extending generally crosswise to the warp fibers, and defining a loft thickness of at least about 0.25", wherein the loft thickness is produced without heat treatment.

These and other aspects, features and advantages of the invention will be understood with reference to the drawing figures and detailed description herein, and will be realized by means of the various elements and combinations particularly pointed out in the appended claims. It is to be understood that both the foregoing general description and the following brief description of the drawings and detailed description of the invention are exemplary and explanatory of preferred embodiments of the invention, and are not restrictive of the invention, as claimed.

#### BRIEF DESCRIPTION OF THE DRAWINGS

FIG. 1 is a perspective view showing the end profile of a turf reinforcement mat according to an example embodiment of the present invention.

FIG. 2 is a plan view of a section of the turf reinforcement mat shown in FIG. 1.

FIG. 3 is a side view in the machine direction showing the end pattern of the turf reinforcement mat shown in FIG. 1.

FIG. 4 is a side view in the cross-wise direction showing the end pattern of the turf reinforcement mat shown in FIG. 1.

FIG. 5 is a chart of the harness pattern for the weave of the reinforcement mat shown in FIG. 1.

FIG. 6 is a harness draw graph showing a harness setup for an example embodiment of the turf reinforcement mat according to the present invention.

FIG. 7 is a schematic view of a loom and take-up roller tensioning system for producing a reinforcement mat according to an example form of the invention.

#### DETAILED DESCRIPTION OF EXAMPLE EMBODIMENTS

The present invention may be understood more readily by reference to the following detailed description of the invention taken in connection with the accompanying drawing figures, which form a part of this disclosure. It is to be understood that this invention is not limited to the specific devices, methods, conditions or parameters described and/or shown herein, and that the terminology used herein is for the purpose of describing particular embodiments by way of example only and is not intended to be limiting of the claimed invention. Any and all patents and other publications identified in this specification are incorporated by reference as though fully set forth herein.

Also, as used in the specification including the appended claims, the singular forms "a," "an," and "the" include the plural, and reference to a particular numerical value includes at least that particular value, unless the context clearly dictates otherwise. Ranges may be expressed herein as from "about" or "approximately" one particular value and/or to

"about" or "approximately" another particular value. When such a range is expressed, another embodiment includes from the one particular value and/or to the other particular value. Similarly, when values are expressed as approximations, by use of the antecedent "about," it will be understood that the particular value forms another embodiment.

In an example form, a manufacturing process according to the present invention creates a turf reinforcement mat or three-dimensional geotextile fabric without the need for the application of heat during the manufacturing process, to produce a woven material having a three-dimensional lofted profile. For example, by selective application of tension in the weaving process and/or control of the weave and fiber arrangement of the product, it has been discovered that a three-dimensional lofted profile can be formed, without the need for application of heat to generate the material's loft. In example embodiments, the material has a thickness or loft of about 0.25 inch or more.

Various types of natural and synthetic yarns can be used to weave the turf reinforcement mat of the present invention, including but not limited to polyethylene, nylon, polyester, PVC, polypropylene, etc. In an example embodiment, the yarn is polypropylene. A monofilament, multi-filament, fibrillated tape or slit tape yarn in various yarn sizes, for example from 400 denier to 3000 denier, can be used to produce a turf reinforcement mat according to the present invention. In an example embodiment, a monofilament having a yarn size of 1675 denier is utilized. The denier of the yarn and the draw ratio used in extruding the yarn provide rigidity to retain loft thickness. An example range of draw ratio is between about 5:0:1 to about 9:0:1 and the value depends upon the yarn denier and required strength. A particular example draw ratio used is 6:0:1. The yarn can be UV stabilized during manufacturing. Coloring is optionally added to the yarn during the extrusion process.

Beams can be made with either direct or sectional warping machines. The number of beam ends is determined by the width of the fabric in conjunction with the machine direction construction on the final fabric. Machine direction construction is determined by the reed that will be used on the loom in the weaving process. The beaming process can be eliminated if a creel is available to be placed behind the loom and weave directly off the yarn packages.

Different weave patterns can be generated on a loom to weave a turf reinforcement mat within the scope of the invention. One example of a weave used is a honeycomb pattern, for example as shown in FIGS. 1-4. An alternative pattern is a tubular weave. The loft and strength of the fabric can be altered and achieved through the use of a variety of yarn sizes and configurations. The size of the yarns used in conjunction with the TRM construction and weave determines the amount of loft as well as the strength of the fabric. Certain strength requirements may be desirable, depending on the intended application of the turf reinforcement mat. The construction and yarn size is modified to decrease or increase the tensile strength of the fabric to meet the requirements. The fabric is of sufficient density to stabilize the soil while still allowing vegetation to grow through the mat. Alternative uses of the material include air filtration and fuel-cell baffles. A mechanical or computer-controlled dobby head is used on the loom to achieve the required weave configuration.

In the example embodiment, the loom setting has a worm gear let-off range of either 3:38 or 2:39 which can be based on the type of mechanical or electronic let-off used on the loom. In conjunction with projectile looms the whip roll setting is in the front position. An example honeycomb weave can be woven on a range of between about 8 and 18 harnesses. The

example embodiment honeycomb is woven on 14 harnesses. FIG. 6 shows a harness weave pattern and FIG. 5 shows a draw graph of the weave pattern according to an example form of the invention. The example embodiment uses a reed on the loom to determine the construction of the fabric by either drawing the ends through the reed dents in one or multiple ends per dent. The example embodiment uses a 23.0 dent per inch reed and the ends are drawn 1 per dent. When coupled with the proper tension settings, the ends per inch, in conjunction with weaving the pick construction into the fabric, provide the appropriate material construction to achieve a desired three-dimensional fabric loft (i.e., the thickness between the top and bottom faces of the material) without the necessity for subsequent heat shrink.

FIGS. 1-4 show an example embodiment of a turf reinforcement material 10 with a honeycomb pattern. The honeycomb pattern is comprised of numerous box-shaped cells or volumes 12, shown in example form in detail in FIG. 2. Each box shaped cell 12 has four sides defining a length L and a width W. The example embodiment has sides defining a width of about 1" and a length of about 1.5", but in alternate forms may vary in length from about 0.5 inch to about 1.5 inches. However, additional sizes outside of this range are within the scope of the invention. Each box shaped cell 12 has a low center or valley 16 in the middle of each of the four sides, and raised corners or peaks 18 at the intersections of the sides of the cell. Each box shaped cell 12 has angled walls from the sides to the center 16, and each angled wall has a triangular shape. Otherwise described, each cell of the matrix of cells in the pattern defines an alternating and repeating upright and inverted pyramid-shaped profile formed by the intersections of the fibers within the weave.

Each box shaped cell 12 is created by weaving warp (machine direction) 20 and weft or fill (cross-machine direction) 22 filaments in a perpendicular weave pattern and manner with respect to each other. At the peaks and valleys 16 of each box shaped cell 12, a plurality of fill filaments 22 are set on top of a central warp filament 20 in perpendicular or crosswise relation with respect to each other, forming alternating upper and lower crests (e.g., ridges and valleys in at least one of the warp and/or weft filament patterns) in the machine and cross-machine directions. Provision of a plurality of fill filaments 26 at the crests provides increased resistance to compression of the material in use. In the depicted embodiment, three crest filaments 26 are utilized, but in alternate embodiments, one, two or more than three crest filaments are provided. Also, while the depicted embodiment provides multiple crest filaments 26 in the fill direction, alternate embodiments may comprise multiple crest filaments in the warp direction or in both the warp and fill directions at the peak and/or valley boundaries of each cell 12 of the turf reinforcement material 10. Two horizontal filaments are then set on top of the vertical filament on either side of the central horizontal filament and each parallel to the central horizontal filament. Two vertical filaments are then set on top of the horizontal filaments on either side of the central horizontal filaments and parallel to the central horizontal filament. This process is repeated with further horizontal filaments extending further from, and parallel to, the central horizontal filament and with further vertical filaments extending further from, and parallel to, the central vertical filament, until the height 24 from the center 16 to each corner is at least about 0.25 inches as shown in FIG. 4. The number of filaments can vary depending on the thickness of each filament and the distance between the parallel filaments. The final vertical and horizontal filaments applied to the honeycomb pattern define the sides of each box shaped cell 12. An example embodiment has about twenty-four warp

filaments 20 and twenty weft filaments 22 per box shaped cell 12. In alternate embodiments, more or fewer filaments per cell are provided.

In the example embodiment, each filament has the same tensioning level and warp level, and the same yarn stiffness and denier. In alternate embodiments, varying tensioning, warp level and/or yarn characteristics are within the scope of the invention. The harness operation is preferably automatically controlled, for example by electronic or punch card programming. FIG. 5 is a harness draw graph for setting up the loom harnesses to generate the three-dimensional basket-weave pattern of the depicted example. FIG. 6 is a harness weave pattern chart showing the harness positions at sequential shuttle passes during the weave process. Yarns of a specified stiffness and denier are drawn in through the harnesses and reed per the draw graph, the harnesses are installed onto the loom, and the loom is operated in typical fashion to produce the TRM material. The weave pattern and manufacturing method result in a three-dimensional TRM material having a thickness or loft substantially greater than the fiber thickness, and preferably at least about 0.25 inches, as seen best with reference to FIG. 3, without the need for application of heat to produce the loft.

FIG. 7 shows a tension roller system 100 for tensioning the turf reinforcement mat 102 as it is drawn off the loom 110. A packer roller 112 and a pulling roller 114 are driven by a motor via a chain and sprocket drive, with the tooth ratio of the rollers selected as shown to apply tension as the turf reinforcement mat is collected in a product roll 120. A deflection roller 116 directs the mat 102 from the loom 110 to the packer roller 112.

While the invention has been described with reference to preferred and example embodiments, it will be understood by those skilled in the art that a variety of modifications, additions and deletions are within the scope of the invention, as defined by the following claims.

What is claimed is:

1. A three-dimensional turf-reinforcement fabric comprising a woven array of fibers comprising a first plurality of warp fibers arranged in a first direction and a second plurality of weft fibers arranged in a second direction generally perpendicular to the first direction, wherein the second plurality of weft fibers are interwoven with the first plurality of warp fibers to form an interlaced weave of warp and weft fibers, the woven array of fibers defining rows and columns of cells, wherein each cell comprises fiber segments of the first plurality of fibers and the second plurality of fibers being spaced at differing heights in a third direction perpendicular to the first and second directions, wherein the three-dimensional turf-reinforcement fabric is formed without the application of heat to produce a loft.

2. The three-dimensional turf-reinforcement fabric of claim 1, wherein the woven array of fibers comprises a tubular or honeycomb pattern.

3. The three-dimensional turf-reinforcement fabric of claim 1, wherein the fibers are selected from polypropylene, polyethylene, nylon, polyester, PVC, other natural or synthetic fibers, and combinations thereof.

4. The three-dimensional turf-reinforcement fabric of claim 1, wherein the loft of the fabric is produced by control of at least one of the following parameters: loom tension setting, ends per inch of the weave, and weaving the pick construction into the fabric.

5. The three-dimensional turf-reinforcement fabric of claim 1, wherein the cells comprise alternating upper and lower crests defining a material thickness in the third direction therebetween.

6. The three-dimensional turf-reinforcement fabric of claim 5, wherein the first plurality of fibers arranged in the first direction comprise a plurality of fibers at each of the upper and lower crests.

7. The three-dimensional turf-reinforcement fabric of claim 5, wherein the material thickness is at least about 0.25".

8. A method of forming a three-dimensional turf-reinforcement fabric, said method comprising weaving a first plurality of warp fibers arranged in a first direction and a second plurality of weft fibers arranged in a second direction generally perpendicular to the first direction into a woven array of interlaced warp and weft fibers interwoven with one another, and having fiber segments being spaced at differing heights in a third direction perpendicular to the first and second directions, using a loom, without the application of heat to produce a loft.

9. The method of claim 8, further comprising controlling at least one of a loom tension setting, ends per inch of the weave, and/or weaving the pick construction into the fabric.

10. The method of claim 8, wherein the first plurality of fibers arranged in the first direction comprise a plurality of fibers arranged at alternating upper and lower crests of the fabric.

11. The method of claim 8, further comprising weaving the first plurality of fibers and the second plurality of fibers into a modified honeycomb weave having 3 fiber ends at each peak and valley of said weave along at least one of the first and second directions.

12. The method of claim 8, further comprising weaving the first plurality of fibers and the second plurality of fibers into a turf-reinforcement fabric having a loft of at least about 0.25".

13. The method of claim 8, further comprising controlling the off-loom take-up tension of the turf-reinforcement fabric as it is rolled after weaving.

14. The method of claim 8, wherein the loft is produced without the three-dimensional turf-reinforcement fabric shrinking in the first or second directions after weaving.

15. A turf reinforcement mat comprising a weave formed of a plurality of warp fibers, a plurality of weft fibers extending generally crosswise to the warp fibers and interwoven therewith to form an interlaced weave of warp and weft fibers, and defining a loft thickness of at least about 0.25", wherein the loft thickness is produced without heat treatment; and the weave is a modified honeycomb weave defining alternating peaks and valleys, the weave further comprising a plurality of crest fibers of at least one of the warp and weft fibers at the peaks and valleys to resist compression of the loft thickness.

16. The turf reinforcement mat of claim 15, wherein the weave comprises a matrix of cells arranged in rows and columns, each of the cells comprising a three-dimensional pyramid-shaped fiber array.

17. The turf reinforcement mat of claim 15, wherein the fibers comprise polypropylene.

18. The turf reinforcement mat of claim 15, wherein the weave comprises at least 20 ends per inch in at least one of the warp and weft directions.

19. The turf reinforcement mat of claim 18, wherein the weave comprises 23 ends per inch in at least one of the warp and weft directions.

\* \* \* \* \*